

## UNITED STATES PATENT OFFICE.

ARTHUR PERCY STROHMEGER, OF LONDON, ENGLAND, ASSIGNOR TO THE QUASI-ARC COMPANY LIMITED, OF LONDON, ENGLAND.

## WELDING ELECTRODE.

No Drawing. Application filed June 17, 1926, Serial No. 116,730, and in Great Britain September 16, 1925.

This invention relates to electrodes such as are employed in the fusion deposition of metals by the process known as "arc welding" and for cutting or preparing metal surfaces preparatory to welding or other operations.

For many years past it has been realized that in order to effect electric welding with the deposition of fused metal the deposit should be as free as possible from oxide or other impurities. It is of great importance to select a suitable covering material for the metallic electrode which shall form a slag during the welding operation and will tend to remove impurities from the metal while also protecting the metal from oxidation during deposition and cooling. Various forms of covering materials have been proposed and used from time to time for this purpose, some of these being applied as a paste, while in recent years other forms of coverings have been developed, one which has had a very large use being a covering of blue asbestos yarn or fibre wound spirally around the electrode. It has been recognized that blue asbestos contains a substantial proportion of iron in the form of ferrous silicate, and its favourable effects have been attributed to the reducing action which iron in the ferrous state is capable of exerting in the slag. In order to increase this effect, aluminium or an equivalent material having a high affinity for oxygen has been used, generally wound in with the covering in the form of a wire, strip or plating on the metallic core of the electrode, and electrodes made in this manner, as described for example in the specification of my United States Patent No. 1,144,390, have been very successful in practice.

I have found, in comparing the results obtained from electrodes covered with various mixtures of blue asbestos with white asbestos and other materials, that the higher the percentage of iron, that is to say the nearer the covering material is to being pure blue asbestos of high iron content, the more effective in general is the slag covering in producing the results desired. These results, however, depend according to my research not only upon the reducing action

of the slag which melts with the core of the electrodes during the welding, and covers the surface as the welding progresses, but also upon the various other characteristics of the slag material. For example, it is most important that the slag should flow evenly and regularly over the surface of the molten metal covering it completely, and forming a layer of sufficient thickness to insure that the rate of cooling of the metal deposited will be favourable to the ultimate structure of the weld junction between the deposited metal and the body of the metallic article on which the deposit is being effected. The fusion temperature of the covering material is also important, and the fusion temperature of blue asbestos has been found to make it more suitable as a covering material for electrodes than most other substances, while the possibility of applying it spirally around the electrode as a yarn is a matter of very great practical importance because it insures the even and regular fusion of the covering as the electrode core melts.

The slag resulting from some covering materials does not fuse evenly as the electrode core is melted, and the slag forms an indifferent or irregular covering on the surface of the deposited metal, with the result that not only is oxidation liable to occur, but the metal cools in such a way that the junction between the welding metal and the metallic structure to which it is applied is liable to have a coarse crystalline formation which tends to produce serious weaknesses in this zone. Welds made with blue asbestos as a covering material upon the electrodes are strikingly superior to welds made with other kinds of slags applied to the electrode, but the research has shown that there is room for further improvement in this respect. Attempts to increase the amount of iron by incorporating a solid ferrous oxide in the covering material, have not proved successful, possibly because of the necessity of applying such material as a paste involving other constituents which render the added oxide of iron ineffective for the purpose in view.

I have now found that it is possible to

attain the desired result with the use of minerals other than crocidolite, but which occur in a long crystalline or fibrous form and which contain a higher percentage of iron. One of these minerals is a variety of hornblende known as "amosite." Whereas crocidolite contains generally from 24 to 28% or thereabouts of iron, amosite contains generally well over 30% of iron, and sometimes nearly 40%. It is essentially an iron silicate but the proportion of ferrous to ferric oxide in its composition is liable to vary substantially. In experiments which I have made with this material, using it alone or in a mixture with blue asbestos as a covering for electrodes I have discovered that it has substantial advantages over any other covering material, not only in the directions mentioned already but in other respects, as hereinafter set forth. The slag resulting from this material has a high iron content and its coefficient of expansion is substantially different from that of deposited metal, with the result that as the metal cools, the slag covering tends to separate from the deposit, and is easier to remove than the slag resulting from blue asbestos alone. The slag formed does not tend to separate from the deposited metal until this latter has cooled down to a point well below that at which there is risk of oxidation, probably about from 200° to 150° C., so that the surface of the metal deposited is not deleteriously affected even if the slag flies off on its own account at or below this temperature. The improvement in the crystal-structure at the weld joint when the covering material contains the higher iron content is most marked, the crystals as shown by photomicrographs of sections of the weld at the weld junction being comparatively small and very uniformly distributed. I can only attribute this result to an improved annealing effect due to the use of this new covering material.

Although amosite, when used as the main constituent of the covering material, has all the advantages set forth, yet certain incidental difficulties arise in connection with its use. Amosite fibres are found to be considerably more brittle than those of blue asbestos, so that the material is more difficult to card and to spin into yarn. Further, when amosite is used as the covering material, the slag is more viscous than that from blue asbestos, probably owing to its high iron content, and this renders the operation of welding with amosite-covered electrodes rather more difficult. The operator has to be particularly careful to avoid trapping slag in the weld metal. For these reasons I prefer to use a mixture of blue asbestos and amosite fibres, which can be carded and spun together, the spun mixture being very suitable for use as an electrode

covering material. It has the requisite strength for winding, and the slag flows more freely so that welding is facilitated, and the results are more uniform and reliable. I find that a mixture of about equal parts of blue asbestos and amosite is very suitable for all purposes, as the yarn has the necessary strength, the addition of the amosite substantially increases the iron content in the slag, and the welds have a high resistance to fracture, as tested by alternating impact and bending stresses, or in any other effective manner.

Although amosite has been referred to as the material preferably used to increase the iron content of the electrode covering, it is to be understood that any mineral consisting essentially of silicate of iron crystals in a long fibrous form, so that it can be spun into yarn or otherwise applied as a fibrous covering to the core of an electrode, may be used provided that its percentage content of iron is sufficient for the purpose in view. The improvements which I have noted are most marked when forms of amosite containing from 35% of iron upwards are used, but a substantial improvement over anything obtainable with blue asbestos and other covering materials alone is noticeable even when the iron content of the covering material is but little more than 30%. The covering material or mixture of materials is preferably spun into yarn and applied to the electrode core by winding spirally thereon with the use of sodium silicate or other material of a similar character to secure the turns of the yarn upon the electrode and to make a paste or cement which may be added to by impregnating the electrode with any other materials in solution or suspension. Although it is preferable to apply the material as a yarn, the fibrous material may be lapped around the electrode in any suitable manner, and the invention is not limited to spinning the material into yarn before its application.

The invention is also not limited to the use of electrodes covered with amosite alone or mixtures thereof with blue asbestos, for the deposition of iron and steel, as the same covering material may be employed for electrodes made of any of the metals which are capable of being deposited by fusion deposition.

Further, electrodes of the character set forth can be used for cutting metal either for severing the same or for clearing out a space preparatory to welding.

Having thus described my invention what I claim as new and desire to secure by Letters Patent is:—

1. An electrode adapted for use in the welding and cutting of metals, comprising a metallic core with a covering of fibrous material wrapped around it, said fibrous

material consisting essentially of a mixture of fibrous crocidolite and amosite in the proportion of about one-half each.

2. An electrode adapted for use in the welding or cutting of metals comprising a metallic core with a covering in the form of a composite yarn wrapped spirally there-

on, said composite yarn consisting of a mixture of fibrous crocidolite and amosite so proportioned that the iron content is between 30 and 40 per cent.

In witness whereof, I hereto subscribe my name this 7th day of June, A. D. 1926.

ARTHUR PERCY STROHMEYER.